

Feb. 7, 1950

W. E. BLACKBURN

2,496,432

SELENIUM RECTIFIER

Filed May 21, 1946



WITNESSES:

Edward Michaels  
Mrs. L. Groome

INVENTOR

Wayne E. Blackburn.

BY

F. W. Lyle.  
ATTORNEY

## UNITED STATES PATENT OFFICE

2,496,432

## SELENIUM RECTIFIER

Wayne E. Blackburn, Wilkinsburg, Pa., assignor  
to Westinghouse Electric Corporation, East  
Pittsburgh, Pa., a corporation of Pennsylvania

Application May 21, 1946, Serial No. 671,176

## 4 Claims. (Cl. 175—366)

1

My invention relates to selenium rectifiers, and, in particular, relates to an improved method of rendering the junction between the selenium and the counterelectrode unilaterally conductive. A number of different procedures for improving the unilateral nature of the above-mentioned junction have been employed in the prior art, such procedures being commonly referred to as the production of the blocking layer at the selenium surface.

One object of my invention is, accordingly, to provide an improved type of selenium rectifier.

Another object of my invention is to provide an improved type of blocking layer for selenium rectifiers.

Still another object of my invention is to produce a blocking layer for selenium rectifiers, which is particularly effective in withstanding high inverse voltages.

Other objects of my invention will become apparent upon reading the following description, taken in connection with the single figure of drawing which is a cross-sectional view of a selenium rectifier embodying the principles of my invention.

Referring to the drawing, a suitable form in which the principles of my invention may be embodied comprises a base plate 1 which may be of steel, and which is preferably nickel-plated and sand-blasted on the surface. One face of the plate 1 is coated with a layer 2 of selenium which may be applied by dipping the plate 1 in a molten bath of selenium, and thereafter rotating the plate on a suitable spindle, or other device, to throw off the excess of selenium, while molten, by centrifugal force. The free surface of the selenium is then coated, in accordance with my invention, with a thin film 3 of one of the following metals: germanium, silicon, magnesium, aluminum, cerium, beryllium, indium. This thin layer of one of the above metals may, for example, be applied by vaporizing the metal and condensing it in an evacuated container. The film is preferably made thin enough to permit diffusion through it by the materials of a counterelectrode 4 which is subsequently applied by metal spraying cadmium, or an alloy of cadmium and tin. For example, the thickness of the above-mentioned thin film of metal may be about one micron.

After deposition of the counterelectrode 4, the unit is heat-treated at a temperature of about 200° C. for a period of about 2 hours. The unit may then be "electrically formed" by impressing,

between the terminals 1 and 4, a self-rectified sixty-cycle voltage of about 30 volts for a period of about one hour. Thereupon, the element is suitable for use in any of the standard connections of rectifier units well-known in the art.

5 I claim as my invention:

1. The method of improving the unilaterally-conductive properties of the junction between the selenium and the counterelectrode in a se-

10 lenium rectifier which comprises superposing a thin layer of metal selected from the group consisting of magnesium, aluminum and beryllium on the surface of the selenium and superposing on said layer a counterelectrode contain-

15 ing cadmium.

2. The method of producing a conducting element for electric circuits which comprises coating a base plate of metal with a layer of selenium, coating the free surface of the selenium with a thin layer of one or more metals selected from the group consisting of magnesium, aluminum and beryllium, depositing a layer containing cadmium on the free surface of said layer, and heat-treating the unit thus formed.

25 3. An electric circuit element comprising a base plate having a layer of selenium deposited on a portion of its surface, a thin layer of one or more metals selected from the group consisting of magnesium, aluminum and beryllium and a counterelectrode containing cadmium superposed on the free surface of the last-mentioned layer.

30 4. An electric circuit element comprising a base plate having a layer of selenium deposited on a portion of its surface, a layer of one or more metals selected from the group consisting of magnesium, aluminum and beryllium and a counterelectrode containing cadmium superposed on the free surface of the last-mentioned layer,

35 40 said layer being thin enough to permit diffusion through it by materials from said counterelectrode.

WAYNE E. BLACKBURN.

## 45 REFERENCES CITED

The following references are of record in the file of this patent:

## UNITED STATES PATENTS

| 50 | Number    | Name           | Date          |
|----|-----------|----------------|---------------|
|    | 2,096,170 | Geisler -----  | Oct. 19, 1937 |
|    | 2,361,157 | Thompson ----- | Oct. 24, 1944 |
|    | 2,380,880 | Thompson ----- | July 31, 1945 |